

May 29, 1928.

1,671,490

H. SCOTT

BIMETAL ELEMENT

Filed Dec. 27, 1926



WITNESSES:

E. G. McElroy.  
G. B. Goflat

INVENTOR

Howard Scott.

BY

Wesley G. Barr  
ATTORNEY

Patented May 29, 1928.

1,671,490

# UNITED STATES PATENT OFFICE.

HOWARD SCOTT, OF WILKINSBURG, PENNSYLVANIA, ASSIGNOR TO WESTINGHOUSE ELECTRIC & MANUFACTURING COMPANY, A CORPORATION OF PENNSYLVANIA.

## BIMETAL ELEMENT.

Application filed December 27, 1926. Serial No. 157,321.

My invention relates to thermostatic devices and particularly to bimetallic elements therefor.

An object of my invention is to provide a bimetallic element for a thermostatic device that shall have uniform and high temperature deflection characteristics over a predetermined range of temperature.

Another object of my invention is to provide a bimetallic element for a thermostatic device that shall have temperature deflection characteristics from low temperatures to above 300° C. similar to that of a bimetal having brass for the expanding element, but having greater strength at high temperatures than a brass bimetallic element.

In practicing my invention I provide a bimetallic element for a thermostatic device in which the metal having the low temperature coefficient of expansion is an alloy of nickel and iron and the cooperating metal therefor is an alloy of manganese, nickel and iron. The manganese-nickel-iron alloy has a high temperature coefficient of expansion that is uniform over a relatively wide range of temperatures, say from -100° C. to +500° C.

A bimetal composed of two metallic alloys, one of which is nickel steel and the other which is manganese, nickel and iron, is very sensitive to temperature changes, particularly at temperatures to which bimetal is ordinarily subjected.

In the single sheet of drawings, the temperature expansion characteristics of a ferrous alloy containing manganese and nickel and a second ferrous alloy containing nickel are illustrated diagrammatically by means of curves. The difference in expansion between these alloys, which is a measure of the deflection at any temperature that can be obtained when these alloys are joined into a bimetallic strip, is also plotted.

In the drawings the ordinates of the curves represent deflection in thousandths per unit length per degree centigrade and the abscissæ represent temperature in degrees centigrade.

Curve 11 represents the temperature expansion characteristics of a ferrous alloy containing approximately equal parts of manganese and nickel in substantial quantities. Curve 12 represents the temperature

expansion characteristic of a relatively low expansion ferrous alloy that contains approximately 38% nickel and curve 13 represents the temperature deflection characteristic of a bimetal composed of the alloys represented by the curves 11 and 12. The ordinates of curve 13 are obtained by subtracting 60 the ordinates of curve 12 from the ordinates of curve 13.

While I have designated a ferrous alloy containing 38% nickel as the low expansion element of my improved bimetallic element, 65 I do not wish to be limited to the use of this alloy as other alloys having a low temperature coefficient of expansion may be employed. When using a ferrous alloy containing nickel, the nickel content may be as 70 high as 45% if so desired.

It is to be noted that the alloy represented by the curve 11 is concave upwards from -150 to approximately -75° C. and from -75° C. to +450° C. the curve is substantially a straight line, the regularity of which indicates that the alloy composed of manganese, nickel and iron expands substantially uniformly over the temperature range from -75° C. to +450° C. 75

The curve 12 represents approximately a 38% nickel iron alloy that cooperates with the alloy represented by curve 11 and it is to be noted that the expansion characteristic of the nickel iron alloy is substantially uniform 85 between -100° C. to substantially +250° C.

The temperature expansion characteristics of a bimetal composed of the alloys represented by the curves 11 and 12 is particularly illustrated by curve 13. It is to be 90 noted that bimetal composed of these alloys has substantially uniform deflection from -75° C. to substantially +250° C. At temperatures higher than 300° C. the bimetal deflects at a lower rate than it does between 95 -100° C. and 300° C. and the curve approaches the horizontal, indicating that the deflection decreases with further increases of temperature.

The temperature range for a uniform deflection coefficient characteristic of the temperature deflection coefficient between 0° C. and 250° C. can be extended to temperatures higher than 250° C. Thus, a bimetal composed of the alloy of curve 11 and an alloy 105 having a higher nickel content than the alloy

of curve 12 will have a straight line deflection characteristic from  $-100^{\circ}$  C. to a temperature higher than  $+300^{\circ}$  C., depending on the increase in nickel of alloy corresponding to curve 12.

If pure iron is heated gradually to high temperatures, and the expansion thereof is recorded, it will be found that it expands quite uniformly up to about  $900^{\circ}$  C., at 10 which temperature, the metal undergoes a change in crystalline structure known as a "transformation point" of the iron. Up to  $900^{\circ}$  C. the crystalline structure of the iron is commonly known as "Alpha" iron. From 15  $900^{\circ}$  C. to  $1400^{\circ}$  C. pure iron expands uniformly but at a much higher rate than it does at temperatures below  $900^{\circ}$  C. The increased coefficient of expansion between the temperatures  $900^{\circ}$  C. and  $1400^{\circ}$  C. is attributable 20 to a new crystalline structure commonly known as Gamma iron or Austenite. The temperature coefficient of expansion of "Austenitic" iron is substantially  $20 \times 10^{-6}$  centimeters per  $^{\circ}$  C. Above  $1400^{\circ}$  C. the 25 structure of the iron changes to that known as Delta iron.

I have found that by adding an appreciable amount of manganese to pure iron the temperature expansion characteristic of 30 "Austenitic" iron may be obtained at low temperatures, say between  $-100^{\circ}$  C. and  $+400^{\circ}$  C. An addition of nickel, or some other alloying element that has the same effect, to the alloy, the characteristics of 35 which are illustrated by curve 11, is used to raise the Gamma to Delta transformation above the proposed range of temperatures. Since the manganese is not as expensive as nickel it is desirable to use manganese as 40 the predominating alloying element so far as other characteristics of the alloy will permit.

Manganese in sufficient quantity lowers the 45 temperature of the irreversible transformation of Alpha to Gamma to temperatures below normal, but also brings the other irreversible transformation of iron, Gamma and Delta, within the desired working range. The function of the nickel is to raise this latter transformation above the working range. Thus with 10% nickel, the high expansion 50 characteristic of Austenite or Gamma iron is available over a temperature range between at least  $-100^{\circ}$  C. to  $+400^{\circ}$  C. Curve 55 11 gives the expansion characteristic of such an alloy.

It is desirable that the manganese content plus two and one half times the nickel content shall not be less than 30%. The 60 amounts of nickel and manganese may be present in larger quantities provided that the general temperature characteristics of the alloy represented by the curve 11 do not depart materially therefrom. I have found 65 that a ferrous alloy, of the character here

referred to, containing 10% manganese, and 10% nickel is particularly responsive to changes in temperature and has a uniform temperature expansion characteristic.

I have provided a bimetallic element that 70 is composed of ferrous alloys, the high expansion member of which is a manganese-nickel-iron alloy and the other of which is a nickel iron alloy. The bimetal has a uniform temperature expansion characteristic 75 from temperatures below zero degrees C. to above  $250^{\circ}$  C. The temperature expansion range of this bimetal may be varied by increasing or decreasing the nickel content of the nickel-iron alloy. The temperature expansion characteristics of the bimetal may 80 also be varied in accordance with the application to which it is to be adapted by varying either or both the manganese and nickel content in the iron-nickel-manganese and 85 the nickel content in the iron-nickel alloy.

Various modifications may be made in the device embodying my invention without departing from the spirit and the scope thereof. I desire therefore that only such limitations shall be placed thereon as are imposed 90 by the prior art and the appended claims.

I claim as my invention:

1. A thermostatic element comprising a pair of metallic elements having different 95 temperature coefficients of expansion, one of said elements being a ferrous alloy containing substantially 15% manganese, and the other of said elements being a nickel-iron alloy.

2. A thermostatic element comprising a pair of metallic elements having different temperature coefficients of expansion, one of 100 said elements being a ferrous alloy containing substantially equal parts of nickel and manganese, and the other of said elements being a nickel-iron alloy.

3. A thermostatic element comprising a pair of metallic elements having different 105 temperature coefficients of expansion, one of said elements being a ferrous alloy containing manganese and nickel in such proportions that the nickel content plus substantially two and one-half times the manganese content is not less than substantially 110 thirty per cent of the alloy aggregate, and the other of said elements being a nickel-iron alloy.

4. A thermostatic element comprising a pair of metallic elements having different 115 temperature coefficients of expansion, one of said elements being a ferrous alloy containing nickel and manganese, the manganese content being not less than 8%, and the other of said elements a nickel-iron alloy.

5. A thermostatic element comprising two 120 cooperating metals having different temperature coefficients of expansion, one of said elements being a ferrous alloy containing nickel and manganese, the manganese con-

tent being not more than 15% of the alloy aggregate, and the other of said elements being a nickel-iron alloy.

6. A thermostatic element comprising two cooperating metals having different temperature coefficients of expansion, one of said elements being a ferrous alloy containing substantially 10% nickel and 10% manganese, and the other of said elements being a nickel-iron alloy.

7. A thermostatic element comprising two cooperating metals having different temperature coefficients of expansion, one of said elements being a ferrous alloy containing nickel and manganese, and the other of said elements being a nickel iron alloy.

8. A thermostatic element comprising two cooperating metals having different temperature coefficients of expansion, one of said elements being a ferrous alloy containing nickel and manganese, and the other of said elements being a nickel-iron alloy having a nickel content of from substantially 38% to 45%.

9. A thermostatic element comprising two cooperating metals having different coefficients of expansion, one of said metals being a ferrous alloy containing nickel and manganese, and the other metal being a ferrous alloy containing 38% of nickel.

10. A thermostatic element comprising two cooperating metals having different coefficients of expansion, one of said metals being a ferrous alloy containing nickel and manganese, and the other metal being a ferrous alloy containing nickel not in excess of 45%.

11. A thermostatic element comprising two cooperating metal elements, one of said elements being a ferrous alloy having a nickel content of from 38 to 45%, the other element being a ferrous alloy containing manganese and nickel in such proportions that the percent amount of manganese plus substantially two and one-half times the percent amount of nickel is not less than substantially thirty percent of alloy aggregate.

12. A thermostatic element comprising two cooperating metal elements, the low expansion element being a ferrous alloy containing substantially 38% nickel, and the high expansion element being a ferrous alloy containing substantially ten percent of manganese and ten percent of nickel.

In testimony whereof, I have hereunto subscribed my name this 21st day of December, 1926.

HOWARD SCOTT.